



US010480054B2

(12) **United States Patent**  
**Valdez et al.**

(10) **Patent No.:** **US 10,480,054 B2**  
(b4) **Date of Patent:** **Nov. 19, 2019**

(54) **COILED TUBE WITH VARYING MECHANICAL PROPERTIES FOR SUPERIOR PERFORMANCE AND METHODS TO PRODUCE THE SAME BY A CONTINUOUS HEAT TREATMENT**

(71) Applicant: **Tenaris Coiled Tubes, LLC**, Houston, TX (US)

(72) Inventors: **Martin Valdez**, Buenos Aires (AR); **Bruce A. Reichert**, Houston, TX (US); **Jorge Mitre**, Houston, TX (US)

(73) Assignee: **TENARIS COILED TUBES, LLC**, Houston, TX (US)

(\*) Notice: Subject to any disclaimer, the term of this patent is extended or adjusted under 35 U.S.C. 154(b) by 328 days.

(21) Appl. No.: **14/872,490**

(22) Filed: **Oct. 1, 2015**

(65) **Prior Publication Data**

US 2016/0024625 A1 Jan. 28, 2016

**Related U.S. Application Data**

(62) Division of application No. 13/229,517, filed on Sep. 9, 2011, now Pat. No. 9,163,296.

(60) Provisional application No. 61/436,156, filed on Jan. 25, 2011.

(51) **Int. Cl.**

**C22C 38/38** (2006.01)  
**C21D 8/10** (2006.01)  
**C21D 9/14** (2006.01)  
**E21B 17/20** (2006.01)  
**C21D 6/00** (2006.01)  
**C21D 9/08** (2006.01)  
**C22C 38/02** (2006.01)  
**C22C 38/04** (2006.01)  
**C22C 38/06** (2006.01)  
**C22C 38/26** (2006.01)  
**C22C 38/28** (2006.01)  
**C22C 38/32** (2006.01)

(52) **U.S. Cl.**

CPC ..... **C22C 38/38** (2013.01); **C21D 6/002** (2013.01); **C21D 6/005** (2013.01); **C21D 6/008** (2013.01); **C21D 8/105** (2013.01); **C21D 9/08** (2013.01); **C21D 9/085** (2013.01); **C21D 9/14** (2013.01); **C22C 38/02** (2013.01); **C22C 38/04** (2013.01); **C22C 38/06** (2013.01); **C22C 38/26** (2013.01); **C22C 38/28** (2013.01); **C22C 38/32** (2013.01); **E21B 17/20** (2013.01)

(58) **Field of Classification Search**

None

See application file for complete search history.

(56) **References Cited**

U.S. PATENT DOCUMENTS

|                  |           |                                        |
|------------------|-----------|----------------------------------------|
| 3,316,395 A      | 4/1967    | Lavin                                  |
| 3,316,396 A      | 4/1967    | Lavin                                  |
| 4,163,290 A      | 7/1979    | Sutherlin et al.                       |
| 4,305,059 A      | 12/1981   | Benton                                 |
| 4,491,725 A      | 1/1985    | Pritchard                              |
| 4,629,218 A      | * 12/1986 | Dubois ..... E21B 17/20<br>138/155     |
| 5,191,911 A      | 3/1993    | Dubois                                 |
| 5,328,158 A      | 7/1994    | Lewis et al.                           |
| 6,006,789 A      | 12/1999   | Toyooka et al.                         |
| 6,257,056 B1     | 7/2001    | Shibayama et al.                       |
| 6,527,056 B2     | 3/2003    | Newman                                 |
| 7,182,140 B2     | 2/2007    | Wood                                   |
| 2006/0157539 A1  | 7/2006    | DuBois                                 |
| 2006/0231168 A1  | 10/2006   | Nakamura et al.                        |
| 2008/0115863 A1  | 5/2008    | McCrink et al.                         |
| 2008/0286504 A1  | 11/2008   | Asahi et al.                           |
| 2009/0148334 A1* | 6/2009    | Stephenson ..... C22C 1/1084<br>419/10 |
| 2010/0136363 A1  | 6/2010    | Valdez et al.                          |
| 2011/0259482 A1  | 10/2011   | Peters et al.                          |
| 2011/0284137 A1  | 11/2011   | Kami et al.                            |
| 2012/0186686 A1  | 7/2012    | Valdez                                 |
| 2013/0199674 A1  | 8/2013    | Altschuler et al.                      |
| 2013/0264123 A1  | 10/2013   | Altschuler et al.                      |
| 2014/0057121 A1  | 2/2014    | Altschuler et al.                      |
| 2014/0272448 A1  | 9/2014    | Valdez et al.                          |

FOREIGN PATENT DOCUMENTS

|    |           |         |
|----|-----------|---------|
| CA | 2685001   | 11/2008 |
| CN | 101480671 | 7/2009  |
| EP | 0 788 850 | 8/1997  |
| EP | 2 239 343 | 10/2010 |
| GB | 498472 A  | 1/1939  |

(Continued)

OTHER PUBLICATIONS

Chinese Office Action for Application No. 201210020833.5 with English Translation dated May 5, 2015.

Chitwood, G. B., et al.: "High-Strength Coiled Tubing Expands Service Capabilities", as presented at the 24th Annual OTC in Houston, Texas, May 4-7, 1992, in 15 pages.

European Extended Search Report re EPO Application No. 12152516.6, dated Jun. 25, 2012.

European Search Report and Opinion, re EPO Application No. EP 14159174.3, dated Jul. 3, 2014.

First Chinese Office Action for Application No. 201210020833.5 with English Translation dated Aug. 4, 2014.

(Continued)

*Primary Examiner* — Jenny R Wu

(74) *Attorney, Agent, or Firm* — Fish & Richardson P.C.

(57) **ABSTRACT**

Described herein are coiled tubes with improved and varying properties along the length that are produced by using a continuous and dynamic heat treatment process (CDHT). Coiled tubes can be uncoiled from a spool, subjected to a CDHT process, and coiled onto a spool. A CDHT process can produce a "composite" tube such that properties of the tube along the length of the tube are selectively varied. For example, the properties of the tube can be selectively tailored along the length of the tube for particular application for which the tube will be used.

(56)

**References Cited**

## FOREIGN PATENT DOCUMENTS

|    |                |     |         |
|----|----------------|-----|---------|
| JP | 60-215719      | A   | 10/1985 |
| JP | S60261888      |     | 12/1985 |
| JP | H0574928       |     | 10/1993 |
| JP | H09217120      |     | 8/1997  |
| JP | 2001220653     | A * | 8/2001  |
| WO | WO 2006/078768 |     | 7/2006  |
| WO | WO2006078768   |     | 7/2006  |
| WO | WO 2013/007729 |     | 1/2013  |

## OTHER PUBLICATIONS

- Hollomon, J.H., et al., Time-tempered Relations in Tempering Steel. New York Meeting, pp. 223-249, 1945.
- International Standard Publication. Petroleum and natural gas industries—Materials for use in H<sub>2</sub>S-containing environments in oil and gas production. ANSI/NACE ISO, 145 pages, 2009.
- Pollack, Herman, W., Materials Science and Metallurgy, Fourth Edition, pp. 96 and 97, 1988.
- Tenaris brochure. Coiled Tubes HS80CRA, 2 pages, 2008.
- Tenaris brochure. Coiled Tubes Suggested Field Welding Procedure (GTAW) for Coiled Tubing Grads HS70, HS80, HS90, HS110, 3 pages, 2007.
- Tenaris brochure. Coiled Tubing for Down hole Applications, 10 pages, 2007.
- Savatori et. al. European Commision Report, EUR 2006, EUR2207, 3 pp. STN\_ABSTRACT.

[No Author LIS1ED], "Coiled Tubing String Design," Unknown if this document was publicly disclosed, 2 pages.

[No. Author Listed], "CYMAX Division—Coiled Tubing Reel Sizes," Unknown if this document was publicly disclosed, 1 page.

[No Author Listed], "Orbital TIG Welding Cymax Coiled Tubing," Unknown if this document was publicly disclosed, but dated Nov. 1992, 13 pages.

[No Author Listed], "Southwestern Pipe, Inc.—Cymax Coiled Tubing," Unknown if this document was publicly disclosed, 1 page.

[No Author Listed], "The Development and Testing of CYMAX 100 Coiled Tubing," This document is dated Jan. 1992 and is cited in the bibliography of the Full Body Quenched and Tempered Coiled Tubing dated Mar. 1, 1994, 15 pages.

Faszold et al., "Full-Scale Fatigue Testing With 130K Yield Tubing," Paper SPE-153945, Presented at SPE/ICoTA Coiled Tubing & Well Intervention Conference and Exhibition Jan. 2012, Society of Petroleum Engineers, 6 pages.

Thompson et al., "Full Body Quenched and Tempered Coiled Tubing—Theory vs. Field Experience," Presented at the Second International Conference and Exhibition on Coiled Tubing Technology: Operations, Services, Practices, held at Adams Mark hotel in Houston on or about Mar. 28-31, 1994, Mar. 1, 1994, 20 pages.

U.S. Appl. No. 15/236,056, filed Aug. 12, 2016, Valdez et al.

U.S. Appl. No. 14/190,886, filed Feb. 26, 2014, Valdez et al.

U.S. Appl. No. 15/665,054, filed Jul. 31, 2017, Valdez et al.

U.S. Appl. No. 15/788,534, filed Oct. 19, 2017, Valdez et al.

U.S. Appl. No. 15/943,528, filed Apr. 2, 2018, Valdez et al.

U.S. Appl. No. 15/076,305, filed Mar. 21, 2016, Valdez et al.

\* cited by examiner

*FIG. 1*

FIG. 2





*FIG. 3*



FIG. 4



FIG. 5



FIG. 6

## 1

**COILED TUBE WITH VARYING  
MECHANICAL PROPERTIES FOR  
SUPERIOR PERFORMANCE AND METHODS  
TO PRODUCE THE SAME BY A  
CONTINUOUS HEAT TREATMENT**

INCORPORATION BY REFERENCE TO ANY  
PRIORITY APPLICATIONS

Any and all applications for which a foreign or domestic priority claim is identified in the Application Data Sheet as filed with the present application are hereby incorporated by reference under 37 CFR 1.57.

BACKGROUND OF THE INVENTION

Field of the Invention

Embodiments of the present disclosure are directed toward coiled tubes and methods of heat treating coiled tubes. Embodiments also relate to coiled tubes with tailored or varied properties along the length of the coiled tube.

Description of the Related Art

A coiled tube is a continuous length of tube coiled onto a spool, which is later uncoiled while entering service such as within a wellbore. Coiled tubes may be made from a variety of steels such as stainless steel or carbon steel. Coiled tubes can, for example, have an outer diameter between about 1 inch and about 5 inches, a wall thickness between about 0.080 inches and about 0.300 inches, and lengths up to about 50,000 feet. For example, typical lengths are about 15,000 feet, but lengths can be between about 10,000 feet to about 40,000 feet.

Coiled tubes can be produced by joining flat metal strips to produce a continuous length of flat metal that can be fed into a forming and welding line (e.g., ERW, Laser or other) of a tube mill where the flat metal strips are welded along their lengths to produce a continuous length of tube that is coiled onto a spool after the pipe exits the welding line. In some cases, the strips of metal joined together have different thickness and the coiled tube produced under this condition is called "tapered coiled tube" and this continuous tube has varying internal diameter due to the varying wall thickness of the resulting tube.

Another alternative to produce coiled tubes includes continuous hot rolling of tubes of an outside diameter different than the final outside diameter (e.g., U.S. Pat. No. 6,527,056 B2 describes a method producing coiled tubing strings in which the outer diameter varies continuously or nearly continuously over a portion of the string's length, WO2006/078768 describes a method in which the tubing exiting the tube mill is introduced into a forging process that substantially reduces the deliberately oversized outer diameter of the coil tubing in process to the nominal or target outer diameter, and EP 0788850 describes an example of a steel pipe-reducing apparatus, the entirety of each of which is hereby incorporated by reference, describe such tubes).

These methods described above produce coiled tube having constant properties since the tube is produced with the same material moving continuously through the same process. Therefore, the final design of the produced tube (e.g., dimension and properties) is a compromise between all the tube requirements while in service.

SUMMARY

Described herein are coiled tubes with improved and varying properties along the length. In some embodiments,

## 2

the coiled tubes may be produced by using a continuous and dynamic heat treatment process (CDHT). The resulting new product is a "composite" tube in the sense that the properties are not constant, generating a composite coiled tube (e.g., a continuous length of tube that can be coiled onto a spool for transport and uncoiled for use) with unique and optimized properties. The production of a continuous length of composite coil tube may be performed by introducing a previously produced spool of such product into a continuous and dynamic heat treatment line in order to generate a new material microstructure. The heat treatment is continuous because the tube moves through subsequent heating and cooling processes and it is dynamic because it can be modified to give a constantly changing heat treatment to different sections of the coiled tube.

Continuous coil tube may be made from shorter lengths of flat metal strip which are joined end-to-end, formed into tubular form, and seam welded to produce the starting coiled tube for the process are described herein. The starting coiled tube is thereafter introduced into a CDHT process. The CDHT modifies the microstructure thereby improving properties and minimizing heterogeneous properties between the tube body, the longitudinal weld, and the welds made to join the flat metal strips.

The heat treatment variables can be modified continuously in order to generate different mechanical properties, corrosion resistance properties, and/or microstructures along the length of the coiled tube. The resulting composite coiled tube could have localized increase in properties or selected properties in order to allow working at greater depths, localized increased stiffness to minimize buckling, increased corrosion resistance locally in the areas where exposure to higher concentrations of corrosive environments is expected, or any tailored design that has variation of properties in a specific location.

This variation of properties can result in a minimization or reduction of tapers, improving fatigue life, keeping the internal diameter constant for longer distances, minimizing unnecessary strip-to-strip welds, decreasing weight, improving inspection capabilities, tube volume and capacity among others. In particular, weight can be reduced by having an average wall thickness of the tube less than a tube with tapers since a tapered tube has increased wall thickness in certain regions such as the sections of tube at the top of a well. The outer diameter (OD) of the tapered tube typically remains constant while the inner diameter (ID) of the tube is changed to change the wall thickness. For example, an increase in wall thickness of a section of tube can decrease the ID of the section of tube. Therefore, a tube without tapering can have an ID that is substantially the same throughout the tube. By having a substantially constant ID, the ID along the entire length of tube can be inspected. For example, to inspect the ID, a drift ball can be used. However, the drift ball can only be used to inspect the smallest ID of the tapered tube. In addition, fluid flow rate through a tapered tube (e.g., capacity) is limited to the smallest ID of the tube. Therefore, by not reducing ID in certain sections of the tube by increasing wall thickness, the volume and capacity of the tube can be increased.

In certain embodiments, a method of treating a tube is provided. The method can include providing a spool of the tube, uncoiling the tube from the spool, heat treating the uncoiled tube to provide varied properties along a length of the uncoiled tube, and coiling the tube after heat treating. The varied properties may include mechanical properties. At least one of temperature, soak time, heating rate, and cooling rate can be varied during heat treating of the uncoiled tube

to provide varied properties along the length of the uncoiled tube. In certain embodiments, the tube is heat treated with two or more heat treatments (e.g., a double quench and tempering process). The tube may have a substantially constant wall thickness throughout the tube. The tube may have fewer changes in wall thickness as a result of the varied properties along the length of the tube in comparison to conventional tube without the varied properties to maintain sufficient properties for a particular application.

In certain embodiments, a coiled tube is provided. The coiled tube includes a first substantial portion of the tube having a first set of properties and a second substantial portion of the tube having a second set of properties such that at least one property of the first set of properties is different from at least one property of the second set of properties. For example, the difference between at least one property of the first set of properties and at least one property of the second set of properties can be larger than general variations in at least one property as a result of substantially similar steel composition with substantially similar heat treatment processing. At least one property of the first and second set of properties may include yield strength, tensile strength, fatigue life, corrosion resistance, grain size, or hardness. For example, the first substantial portion of the tube can include a first yield strength and the second substantial portion of the tube can include a second yield strength different (e.g., less or greater) than the first yield strength.

The tube may have fewer changes in wall thickness as a result of the varied properties along the length of the tube in comparison to conventional tube without the varied properties to maintain sufficient properties for a particular application. The tube may have a substantially constant wall thickness throughout the tube. Furthermore, the tube can have a substantially uniform composition throughout the tube. The tube may include a plurality of tube sections welded together and at least a portion of one of the tube sections of the plurality of tube sections comprises the first substantial portion and at least another portion of the same tube section comprises the second substantial portion.

In certain embodiments, a coiled tube for use in a well is provided. The coiled tube can include a continuous length of tube comprising a steel material having a substantially uniform composition along the entire length of the tube. The tube has at least a first portion configured to be positioned at the top of the well and at least a second portion configured to be positioned toward the bottom of the well relative to the first portion. The first portion of tube has a first yield strength and the second portion of tube has a second yield strength, the first yield strength can be different (e.g., greater or less) than the second yield strength. In some embodiments, the first portion has a yield strength greater than 100 ksi or about 100 ksi and the second portion has a yield strength less than 90 ksi or about 90 ksi. In further embodiments, the tube further includes a third portion of tube having a third yield strength between that of the first and second yield strength, the third portion being located between the first and second portions. However, the CDHT allows for the production of numerous combinations of properties (e.g. YS) for any length of pipe.

The tube can have a length of between 10,000 feet and 40,000 feet (or between about 10,000 feet and about 40,000 feet). The first portion of tube may have a length of between 1,000 feet (or about 1,000 feet) and 4,000 feet (or about 4,000 feet). Furthermore, the tube may include a plurality of tube sections welded together, and each of the tube sections may have a length of at least 1,500 feet (or about 1,500 feet).

The length of each tube section is related to the distance between bias welds to form the tube. The tube sections may be welded together after being formed into tubes or may be welded together as flat strips which are then formed into the tube. The tube may have a substantially constant wall thickness. For example, the first portion includes a first wall thickness and the second portion includes a second wall thickness that can be substantially the same as the first wall thickness. The first portion includes a first inner diameter and the second portion includes a second inner diameter that can be substantially the same as the first inner diameter.

In some embodiments, the tube has an outer diameter between 1 inch and 5 inches (or between about 1 inch and about 5 inches). The tube may have a wall thickness between 0.080 inches and 0.300 inches (or between about 0.080 inches and about 0.300 inches). In further embodiments, the tube has a substantially constant wall thickness along the entire length of the tube. The tube may have a substantially constant inner diameter along the entire length of the tube. The tube may have no taperings in some embodiments, while in other embodiments, the tube has at least one taper.

#### BRIEF DESCRIPTION OF THE DRAWINGS

FIG. 1 illustrates an example coiled tube on a spool;  
FIG. 2 illustrates an example rig configured to coil and uncoil tube from a spool;

FIG. 3 illustrates an example of a continuous and dynamic heat treatment process;

FIG. 4 is a flow diagram of an embodiment of a method of using a continuous and dynamic heat treatment process;

FIG. 5 is a plot of Rockwell C hardness (HRC) as a function of maximum temperature for tempering cycles which include heating and cooling at 40° C./sec and 1° C./sec, respectively; and

FIG. 6 is a plot of an example of required mechanical properties for a coiled tube as a function of depth from a well surface (0 ft) to a bottom of the well (22,500 ft) for a 110 ksi tube without being tapered, a four tapered 90 ksi tube, and a six tapered 80 ksi tube; also the dashed line shows mechanical properties for an embodiment of a composite tube without being tapered.

#### DETAILED DESCRIPTION

Described herein are coiled tubes having varying properties along the length of the coiled tube and methods of producing the same. In certain embodiments, a continuous and dynamic heat treatment process (CDHT) can be used to produce coiled tube with varying properties along the length of the coiled tube. The heat treatment is continuous because the tube moves through subsequent heating and cooling processes, and the heat treatment is dynamic because it can be modified to give a constantly changing heat treatment to different sections of the coiled tube.

The heat treatment variables can be modified continuously in order to generate different mechanical properties along the length of the coiled tube. The resulting composite coiled tube can have at least a first portion of the tube having a first set of properties and a second portion of the tube having a second set of properties such that at least one property of the first set of properties is different from at least one property of the second set of properties.

In many applications, the coiled tube will be hanging inside a well and the coiled tube should be strong enough to support the associated axial loads; in other applications, the coiled tube will be pushed inside a well and when removed,

the coiled tube will be pulled against the friction forces inside the well. In these examples, the material of the coiled tube on the top of the well will be subjected to the maximum axial load. In addition, for a deeper well, the wall thickness on the upper part of the coiled tube may be increased in order to withstand the axial load (both from hanging or pulling). The use of tapered tubes has been used to allow increasing wall thickness only in the upper part of the coiled tube in order to reduce the total weight of the coiled tube. Materials of different compositions with higher mechanical properties have also been used in order to increase the resistance of the axial load, but these materials tend to be more expensive, more difficult to process, and have lower corrosion resistance.

In other applications, the coiled tube is pushed inside the well and there may be a requirement for increased stiffness; then the specification for the tube may require increased mechanical properties in order to maximize the stiffness of the coiled tube. In other cases, some areas of the well experience different temperatures and corrosive environments, and the coiled tube is specified with resistance to corrosive environments. Increased corrosion resistance can be produced by decreasing other material properties such as mechanical properties, which is contrary to the objective of increase axial resistance and stiffness.

Coiled tube is used by service companies that will provide a service in one location and then remove the coiled tube, recoil it and move it to a different location. FIG. 1 illustrates an example coiled tube 12 on a spool 14, and FIG. 2 illustrates an example rig 10 that can coil and un-coil coiled tube 12 on a spool 14 and direct the tube 12 into a well. The performance and fatigue life of the tube is related to low cycle fatigue associated with the coiling and un-coiling of the tube in each service operation. The fatigue life is usually reduced in the areas where the flat metal was originally joined. Also, the fatigue life is affected by the mechanical properties and operative conditions of the welding process.

Described herein is a product in which, by a special process, the coiled tube can be produced as a “composite” tube, in which the best properties for each section of the coiled tube are targeted. In this way, the tube properties are tailored along the length of the tube to generate the desired properties in the right place resulting in an overall increase of life due to fatigue, increase in corrosion resistance, and minimization of weight.

The special process (e.g., CDHT) takes advantage of the fact that material properties can be varied with appropriate heat treatments. Since a heat treatment is basically combinations of temperature and time, in a continuous heat treatment process, the temperature and speed (including heating and cooling rates) could be dynamically varied in order to modify the final properties of virtually every section of the tube being treated. Another advantage of the process is that since the final properties are affected by the final temperature and time cycle, the properties of the coiled tube could be fixed (e.g., repaired) if there has been a problem during the process, the heat treatment could be used to refurbish already used coiled tube if severe but reversible damage had occurred, or the heat treatment could be used to change properties of already produced coiled tube. This type of treatment allows the service companies to specify the best coiled tube for a given operation regardless of the number of wells the coiled tube is planned to operate in. If the tailored coiled tube does not find more wells to service and it is obsolete (e.g., the coiled tube does not have properties for available applications), its properties could be changed provided there is no irreversible damage to the coiled tube.

In this way, the process (e.g., CDHT) described herein can generate a unique product (e.g., coiled tube) that could act as new product, new process for operation, and a new service. For example, the unique product can open up the possibility for a new “service” for repairing old coiled tubes or changing properties.

In certain embodiments, a method of treating a tube includes providing a spool of the tube, uncoiling the tube from the spool, heat treating the uncoiled tube to provide varied properties along a length of the uncoiled tube, and coiling the tube after heat treating. FIG. 3 is a schematic that illustrates one embodiment. Tube 12 is uncoiled from a first spool 14a. After being uncoiled, the tube 12 goes through a CDHT process represented by box 20 and is then re-coiled on a second spool 14b.

In certain embodiments, the varied properties include mechanical properties. For example, the mechanical properties can include yield strength, ultimate tensile strength, elastic modulus, toughness, fracture toughness, hardness, grain size, fatigue life, fatigue strength. Many mechanical properties are related to one another such as fracture toughness, hardness, fatigue life, and fatigue strength are related to tensile properties.

The varied properties may include corrosion resistance. Corrosion resistance can include sulfide stress cracking (SSC) resistance. Hydrogen sulfide (H<sub>2</sub>S) dissolves in fluid (e.g., H<sub>2</sub>O), and the corrosive environment can be measured by pH and the amount of H<sub>2</sub>S in solution. Generally, the higher the pressure, the more H<sub>2</sub>S can be in solution. Temperature may also have an effect. Therefore, deeper locations in the well experience higher pressure and higher H<sub>2</sub>S concentrations. As such, corrosion resistance of the tube can be increased along the length of the tube toward the section of tube at the bottom of the well. For example, about the bottom 75% of the well generally has the worst corrosive environment. Therefore, in certain embodiments, the bottom 75% of the length of tube has lower mechanical properties and hence higher corrosion resistance properties than the top 25% of the length of tube.

In general, corrosion resistance is related to mechanical properties. For example, international standard NACE MR0175/ISO 155156 “Petroleum and natural gas industries—Materials for use in H<sub>2</sub>S-containing environments in oil and gas production” in Appendix A (A.2.2.3 for Casing and Tubing), the entirety of which is hereby incorporated by reference, shows a direct correlation of corrosion resistance to mechanical properties. In particular, Appendix A lists some materials that have given acceptable performance for resistance to SSC in the presence of H<sub>2</sub>S, under the stated metallurgical, environmental and mechanical conditions based on field experience and/or laboratory testing. Appendix A indicates that as severity of the environment increases from region 1 to region 3 (increase H<sub>2</sub>S partial pressure and/or pH decreases), the recommendation for maximum yield strength (YS) decreases. For example, for region 1 of low severity YS<130 ksi (HRC<30), for region 2 of medium severity YS<110 ksi (HRC<27) and for region 3 of high severity (HRC<26 or maximum API5CT grade is T95 with HRC<25.4), suitable recommended material in all regions can be Cr—Mo quench and tempered steels.

Table I compares a standard steel product used for a coiled tube that has a ferrite and pearlite microstructure and varying grain size with steel that is quench and tempered. Corrosion resistance of the quench and tempered steel is better than the standard product due to the uniformity of

microstructure. Corrosion resistance of 80 ksi to 110 ksi coiled tube decreases as indicated, for example, in ISO 15156.

TABLE I

| Product Type                                         | Standard Product | Grade 80 (YS ≈ 85 ksi)                                              | Grade 90 (YS ≈ 95 ksi)                                                                            | Grade 110 (YS ≈ 115 ksi) | Corrosion Resistance (due to microstructure)                            |
|------------------------------------------------------|------------------|---------------------------------------------------------------------|---------------------------------------------------------------------------------------------------|--------------------------|-------------------------------------------------------------------------|
| Quench and Tempered Corrosion Resistance (due to YS) |                  | Ferrite + Pearlite + Bainite<br>Grain Size (GS) 80 > GS 90 > GS 110 | Tempered Martensite<br>Carbide Size (CS) 80 > CS 90 > CS 110<br>Dislocation Density 80 < 90 < 110 | High<br>Medium<br>Low    | Low<br>(non-uniform microstructure)<br>High<br>(uniform microstructure) |

During heat treatment, the microstructure will change from ferrite and pearlite to tempered martensite in the case of a quench and tempered process. A microstructure from a quench and tempered process is recommended by NACE for high strength pipes with SSC resistance. Also, carbide refinement due to tempering increases toughness. Localized hardness variations are reduced due to the elimination of pearlite or even bainite colonies that can result from segregation in as-rolled material. Localized increased hardness is detrimental for corrosion resistance. Fatigue life can also be increased by reduction of welds between sections of the tube, improving microstructure of the weld area through heat treatment, and/or reduction of mechanical properties.

A variety of steel compositions can be used in the methods described herein. Furthermore, various steel compositions can be used in the quench and temper process. Steel compositions can include, for example, carbon-manganese, chromium, molybdenum, boron and titanium, or a combination thereof. The steel composition may be selected based on, for example, the line speed, water temperature and pressure, product thickness, among others. Example steel compositions include:

Chromium bearing steel: the coiled tube comprising 0.23 to 0.28 wt. % (or about 0.23 to about 0.28 wt. %) carbon, 1.20 to 1.60 wt. % (or about 1.20 to about 1.60 wt. %) manganese, 0.15 to 0.35 wt. % (or about 0.15 to about 0.35 wt. %) silicon, 0.015 to 0.070 wt. % (or about 0.015 to about 0.070 wt. %) aluminum, less than 0.020 wt. % (or about 0.020 wt. %) phosphorus, less than 0.005 wt. % (or about 0.005 wt. %) sulfur, and 0.15 to 0.35 wt. % (about 0.15 to about 0.35 wt. %) chromium;

Carbon-Manganese: the coiled tube comprising 0.25 to 0.29 wt. % (or about 0.25 to about 0.29 wt. %) carbon, 1.30 to 1.45 wt. % (or about 1.30 to about 1.45 wt. %) manganese, 0.15 to 0.35 wt. % (or about 0.15 to about 0.35 wt. %) silicon, 0.015 to 0.050 wt. % (or about 0.015 to about 0.050 wt. %) aluminum, less than 0.020 wt. % (or about 0.020 wt. %) phosphorus, and less than 0.005 wt. % (or about 0.005 wt. %) sulfur;

Boron-Titanium: the coiled tube comprising 0.23 to 0.27 wt. % (or about 0.23 to about 0.27 wt. %) carbon, 1.30 to 1.50 wt. % (or about 1.30 to about 1.50 wt. %) manganese, 0.15 to 0.35 wt. % (or about 0.15 to about 0.35 wt. %) silicon, 0.015 to 0.070 wt. % (or about 0.015 to about 0.070 wt. %) aluminum, less than 0.020 wt. % (or about 0.020 wt. %) phosphorus, less than 0.005 wt. % (or about 0.005 wt. %) sulfur, 0.010 to 0.025 wt. % (or about 0.010 to about 0.025 wt. %) titanium, 0.0010 to 0.0025 wt. % (or about 0.0010 to

about 0.0025 wt. %) boron, less than 0.0080 wt. % (or about 0.0080 wt. %) N and a ratio of Ti to N greater than 3.4 (or about 3.4); and

Martensitic Stainless Steel: the coiled tube comprising 0.12 wt. % (or about 0.12 wt. %) carbon, 0.19 wt. % (or about 0.19 wt. %) manganese, 0.24 wt. % (or about 0.24 wt. %) Si, 11.9 wt. % (or about 11.9 wt. %) chromium, 0.15 wt. % (or about 0.15 wt. %) columbium, 0.027 wt. % (or about 0.027 wt. %) molybdenum, less than 0.020 wt. % (or about 0.020 wt. %) phosphorus, and less than 0.005 wt. % (or about 0.005 wt. %) sulfur.

Molybdenum could be added to the steel compositions above, and some steel compositions can be combined B—Ti—Cr to improve hardenability. Described in Example 1 in the below examples is a chromium bearing steel.

In certain embodiments, at least one of temperature, soak time, heating rate, and cooling rate is varied during heat treating of the uncoiled tube to provide varied properties along the length of the uncoiled tube.

In certain embodiments, the tube has fewer changes in wall thickness as a result of the varied properties along the length of the tube in comparison to conventional tube without the varied properties in order to maintain sufficient properties for a particular application. The tube may even have a substantially constant wall thickness throughout the tube (e.g., the tube has no tapers). The flat metal strips that are used to form tube sections of the tube can be, for example, between 1,500 feet and 3,000 feet (or about 1,500 feet and about 3,000 feet). Flat metal strips with smaller thickness may be longer than flat metal strips with larger thickness. However, if additional changes in wall thicknesses are desired, the flat metal strips may be shorter to allow for additional changes in wall thickness. Thus, if the length of the flat metal strip needed for each change in wall thickness is shorter than the possible maximum length of the flat metal strip, an extra weld joint is required. As previously discussed, additional weld joints can decrease fatigue life. Therefore, as described herein, the number of weld joints can be decreased by minimizing the number of changes in wall thickness. For example, each tube section can have a length that is maximized. In certain embodiments, the tube does not have a tube section that is less than 1,500 feet long. In further embodiments, the average length of the tube sections is greater than 2,500 feet along the entire length of the tube. In further embodiments, the average length of tube sections is greater than if there were taper changes in the tube.

In certain embodiments, the starting coiled tube is unspooled at one end of the process, then it moves continuously through the heat treatment process and is spooled again on the other end. The spooling devices can be designed to allow rapid changes in spooling velocity, and they can be

moved to follow the coiled tube in order to change the spooling or un-spooling velocity in longitudinal units of tube per unit time even more rapidly (flying spooling).

The CDHT itself can include a series of heating and cooling devices that can easily change the heating and cooling rate of the material. In one example, the material is quenched and tempered dynamically, and FIG. 4 is an example flow diagram of the method 200. The method 200 can include quenching operations, intermediate operations, and tempering operations. In operational block 202, a coiled tube of a starting material is uncoiled. In operational block 204, the tube moves through a heating unit and then, in operational block 206, is quenched with water from the outside. The heating unit can modify the power in order to compensate for the changing mass flow when the tube's outer diameter and wall thickness changes, keeping productivity constant. It can also modify the power if the linear speed is changed when the tempering cycle is adjusted, keeping quenching temperatures constant but final properties different. In operational block 208, the tube can be dried.

The tempering operation can include a heating unit and a soaking unit. For example, in operational block 210, the tube can be tempered, and in operational block 212 the tube can be cooled. The stands of the soaking unit could be opened and ventilated so they can rapidly change the total length (e.g., time) of soaking, and at the same time, they can rapidly change the soaking temperature. At the exit of the soaking line, different air cooling devices can be placed in order to cool the tube to a coiling temperature at which there will not be further metallurgical changes. The control of the temperature and speed allows estimating the exact properties of the complete coiled tube, which is an advantage over certain conventional coiled tubes where testing is performed and properties can be only measured in the end of the spools. In certain conventional coiled tubes, the mechanical properties are estimated from less precise models for hot rolling at the hot rolled coil supplier as well as cold forming process during electrical resistive welding (ERW) forming. In operational block 214, the tube can be coiled onto a spool.

The resulting coiled tube can have a variety of configurations. In certain embodiments, a coiled tube includes a first substantial portion of the tube having a first set of properties, and a second substantial portion of the tube having a second set of properties such that at least one property of the first set of properties is different from at least one property of the second set of properties. Furthermore, the coiled tube may have more than two substantial portions. For example, the coiled tube may have a third substantial portion of tube which have a third set of properties such that at least one property of the third set is different from at least one property of the first set of properties and at least one property of the second set of properties. A substantial portion described herein may be a portion with a sufficient size (e.g., length) to enable measurement of at least one property of the portion. In certain embodiments, at least one property of the coiled tube varies continuously (e.g., near infinite number of portions).

In some embodiments, the first substantial portion of the tube has a first length between 1000 feet and 4000 feet (or between about 1,000 feet and about 4,000 feet), and the second substantial portion of the tube has a second length of

at least 4000 feet (or at least about 4,000 feet). The first and second substantial portions may also have other various lengths.

In certain embodiments, at least one property of the first and second set of properties including yield strength, ultimate tensile strength, fatigue life, fatigue strength, grain size, corrosion resistance, elastic modulus, hardness, or any other properties described herein. Furthermore, a change of mechanical properties (e.g., yield strength) could allow a change in weight of the coiled tube.

In certain embodiments, the tube has fewer changes in wall thickness as a result in the varied properties along the length of the tube in comparison to conventional tube without the varied properties in order to maintain sufficient properties for a particular application. The tube may even have a substantially constant wall thickness throughout the tube.

In certain embodiments, the tube has a substantially uniform composition throughout the tube. For example, the tube may have tube segments that were welded together that do not have significant differences in composition (e.g. tube segments with substantially similar composition). Tube segments can include either (1) tube segments that appear welded together since they were made by welding flat strips, formed into a tube, and welded longitudinally or (2) tube segments that are welded together after being formed into tubes and longitudinally welded.

## EXAMPLES

The following examples are provided to demonstrate the benefits of the embodiments of the disclosed CDHT and resulting coiled tube. For example, as discussed below, coiled tube may be heat treated to provide coiled tube with overall unique properties. These examples are discussed for illustrative purposes and should not be construed to limit the scope of the disclosed embodiments.

### Example 1

As an example, a steel design that is quenched and tempered could include sufficient carbon, manganese and could include chromium or molybdenum or combinations of boron and titanium, and be quenched and tempered at different temperatures. Various other steel compositions such as those described above can also be quenched and tempered in similar methods. In the example below, the coiled tube is comprised of about 0.23 to about 0.28 wt. % carbon, about 1.20 to about 1.60 wt. % manganese, about 0.15 to about 0.35 wt. % silicon, about 0.015 to about 0.070 wt. % aluminum, less than about 0.020 wt. % phosphorus, less than about 0.005 wt. % sulfur, and about 0.15 to about 0.35 wt. % chromium. The amount of each element is provided based upon the total weight of the steel composition.

Laboratory simulations and industrial trials were used to measure the material response to quench and tempering cycles. The lengths were selected to guarantee uniform temperatures (more than 40 feet per condition, the material moved continuously through heating and cooling units in the industrial test and was stationary in the lab simulations). The material was subjected to tempering cycles of different maximum temperatures by heating by induction at 40° C./sec up to the maximum temperature and then cooling in air at 1° C./sec (see FIG. 5 which shows the variation of hardness measured in Rockwell C scale (HRC) of the material as a function of maximum temperature). T1 in FIG.

## 11

5 is a reference temperature (about 1050° F. in this example) that results in a hardness of about 27.5 HRC. The reference temperature and resulting hardness can vary depending on steel composition. These particular cycles did not have a soaking time at the maximum temperature (e.g. the material was not held at the maximum temperature for any significant time), but equivalent cycles at lower temperatures and for longer time could be applied. The material was previously water quenched to the same starting hardness level and to a microstructure composed of mainly martensite (more than 80% in volume).

By applying these tempering cycles, the final properties (e.g. yield strength) could be controlled from 80 to 140 ksi allowing the production of different final products. As indicated by the slope of the hardness as a function of temperature graph in FIG. 5, four points of hardness variation (approximately 11 ksi variation in tensile strength) can be produced if the maximum temperature is varied by more than 70° C. (e.g., hatched triangle in FIG. 5). The tensile strength is related to hardness, and discussion of the relationship can be found, for example, in Materials Science and Metallurgy, by H. Pollack, 4<sup>th</sup> edition, 1988, Prentice Hall, page 96, Table 3; shows that a 22.8 HRC is equivalent to 118 ksi and 26.6 HRC is equivalent to 129 ksi. A hardness difference of 3.8 HRC is 11 ksi in tensile strength. Certain other quench and tempered steels have also been observed to have a similar relationship. This temperature variation is much larger than the control capability of the tempering furnaces, and this example indicates that the tensile strength could be controlled at any point of the tube to much less than a 11 ksi variation. In a standard product without heat treatment, the mechanical properties variation along the length of a hot-rolled coil can be 11 ksi and between coils up to 15 ksi, so the mechanical properties of a standard product may vary along the length of the tube but in an uncontrolled way. In addition, in the standard product, these properties may vary as the tube is formed to different diameters; while in the case of the CDHT tubes these properties can remain constant with chemistry.

As demonstrated, the composite tube produced by a dynamic control of heat treatment process can have precisely selected properties that vary in a controlled fashion in each section of the tube. Calibration curves for the material used in this process allows controlling the exact properties at each location of the tubes by recording the temperature. Similar experiments on other compositions of tube can be used to create calibration curves which can then be used to create process parameters of the CDHT process to produce a coiled tube with select properties along the length of the tube. In addition, tempering models can be used to select processing conditions that could yield select properties along the length of the tube by varying parameters such as time and temperature. For example, Hollomon et al., "Time-temperature Relations in Tempering Steel," Transactions of the American Institute of Mining, 1945, pages 223-249, describes a classical tempering model approach. Hollomon describes that the final hardness after tempering of a well quenched material (high % of martensite) is a function of a time-temperature equation that varies with the type of steel. This model can be used to calculate the final hardness of a material after tempering for any combination of time and temperatures after generating some experimental data. The calibration curves for a tempering process can be generated after the model has been fitted with the experimental data.

## 12

In order to dynamically change the properties, the temperature can be increased rapidly or decreased rapidly using induction heating, air cooling or changing the soaking time (if the cycle of tempering uses temperature and a soaking time and not only temperature as is the case for the example in FIG. 5). This process can be used to generate a unique coiled tube product with varying properties that are changed in order to optimize its use as shown in the examples below. The heat treated microstructure can be much more refined and homogeneous than the hot-rolled microstructure, which can provide improved corrosion and fatigue performance. The heat treatment can also relieve internal stresses of the material, which were generated during forming (e.g., hot-rolling and pipe forming).

## Example 2

20 In certain applications, a coiled tube may be required to operate in wells of up to 22,500 ft deep. The tube minimum wall thickness may be 0.134" and the tube OD may be 2.00". The material may also have good performance in H<sub>2</sub>S containing environments and good fatigue life.

25 If the tube is designed for axial load, without taper changes and with a safety factor of 70%, the material may have a Specified Minimum Yield Strength (SMYS) of at least 110 ksi:

$$0.70 \times \text{SMYS} = A(\text{area}) \times L(\text{length}) \times \text{Density} / A = L \times \text{Density}$$

$$\text{SMYS} = L \times \text{Density} / 0.70 = 22,500 \text{ ft} \times (0.283 \text{ lb/in}^3) \times (12 \text{ in}/\text{ft}) / 0.70 \text{ SMYS} = 110,000 \text{ psi}$$

30 The density value was estimated as the density of iron of about 0.283 lb/in<sup>3</sup>. This indicates that if the tube is designed to have a yield strength of 110 ksi, the cross section at the top of the well will be capable of withstanding the weight of the coiled tube. If the same coiled tube is produced with material having a SMYS of 90 or 80 ksi, it may be necessary to taper the upper length of the coiled tube in order to increase the resistance area "A" (e.g. the wall thickness of the coiled tube is increased in the section closer to the well surface compared to the section of the coiled tube closer to the well bottom. FIG. 6 shows a full line (see the solid lines in FIG. 6) of the required mechanical properties from the bottom of the well (22,500 ft) to the well surface (0 ft) for a 110, 90 and 80 ksi coiled tube. As illustrated in FIG. 6, by performing wall thickness changes (e.g. tapers) (which are generally restricted to a number of standard thicknesses produced by the steel rolling mill), the resulting tapered coiled tube could be built with 110, 90 or 80 ksi material (when the whole coiled tube is manufactured in only one type of material).

35 If a composite coiled tube is defined with the properties varying as indicated by the dotted line in FIG. 6, the well could be serviced since the properties vary to improve the overall performance of the coiled tube as indicated in Table II below. The estimation of relative fatigue life and pumping pressure (calculated relative to the composite coiled tube) in Table II is defined based on models used for prediction of service life and current standards. For example, as illustrated in FIG. 6, the tube can have a yield strength of at least 110 ksi to a depth of about 4,000 feet, a yield strength of at least 90 ksi to a depth of about 6,500 feet and a yield strength of at least 80 ksi at depths greater than about 6,500 feet.

TABLE II

| Example               | # of taper changes | # of weld joints | Internal Flash Removal (Y/N) | Relative weight | Relative pumping pressure | Relative fatigue life | SSC resistance | Cost    |
|-----------------------|--------------------|------------------|------------------------------|-----------------|---------------------------|-----------------------|----------------|---------|
| 110 ksi coiled tube   | 0                  | 9                | Y                            | 100.0%          | 100.0%                    | 80.0%                 | Worst          | Highest |
| 90 ksi coiled tube    | 4                  | 11               | N                            | 103.1%          | 102.8%                    | 53.3%                 | Medium         | Medium  |
| 80 ksi coiled tube    | 7                  | 12               | N                            | 107.5%          | 107.5%                    | 48.9%                 | Best           | Medium  |
| Composite coiled tube | 0                  | 9                | Y                            | 100.0%          | 100.0%                    | 100.0%                | Best           | Lowest  |

Internal flash removal refers to the elimination of the material that is expelled from the weld during the ERW process. This material can only be removed if the taper changes are reduced to zero (e.g. taper changes can restrict or prevent the removal of flash). The presence of the flash can affect the fatigue life as well as the ability to inspect the tube.

The best coiled tube is the composite coiled tube because, while keeping the number of taper changes to zero and the tube weight to a minimum, it has lower mechanical properties down the coiled tube, improving the fatigue life as well as the resistance to embrittlement in H<sub>2</sub>S environments by SSC. Furthermore, the cost of the raw material for the composite coiled tube can be lower. An “all 80 ksi” coiled tube will have similar resistance to SSC but with 7.5% weight increase, while an “all 110 ksi” material will have similar weight and no taper changes but lower fatigue and SSC resistance.

In addition, the number of weld joints between tube sections can be minimized. As shown in Table II, the number of tube sections was higher for 90 ksi coiled tube and 80 ksi coiled tube because of the wall thickness changes (e.g., tapers). The additional tapers can reduce the fatigue resistance of the tube. In certain embodiments, the average length of the tube sections is greater than 2500 feet along the entire length of the tube. In further embodiments, the average length of tube sections is greater than if there were taper changes in the tube.

The composite coiled tube, by minimizing the number of tapers, also increases the coiled tube capacity and volume, as well as reliability of inspection, using a drift ball for example. The internal flash removal with no tapers is also possible if desired.

For a tapered coiled tube, the increased wall thickness reduces the inner diameter and results in higher pumping pressure for the same volumetric flow rate. Higher pumping pressure will both increase the energy required for pumping and reduce the fatigue life by increasing internal stresses. Therefore, the composite product described herein can have optimized properties and improved properties over a tapered coiled tube.

Pumping pressure can be a function of tube length and inside diameter, and pumping pressure can be calculated using well-known fluid mechanics relationships. Therefore, by increasing the inside diameter of the tube, the pumping pressure can be reduced for a certain flow rate. Furthermore, fatigue life can be affected by many factors including the tube yield strength, the internal pressure, and others. The example tubes described herein can have improved fatigue life by having a combined effect of selecting yield strength, decreasing internal pressure (e.g., pumping pressure), and decreasing number of strip to strip welds. SSC resistance can

15 be assessed in accordance with NACE TM0177 and NACE MR0175. One strong correlation in C—Mn steels is the relationship between hardness and SSC resistance. As previously discussed, in general, steel with a higher hardness results in lower SSC resistance. Also in general, steel with a higher strength has a higher hardness which results in a lower SSC resistance. The composite coiled tube can have lower strength tube confined to the lower part of the coiled tube where the SSC exposure is higher. Furthermore, the composite coiled tube can have high strength tube confined to the upper part of the coiled tube where the SSC exposure is less.

20 The properties after a heat treatment are affected by the time and temperature history of the material, making the process subject to validation. The validation process is supported by metallurgical models that allows for the correct prediction of tube properties at each section of the coiled tube. In the certain conventional coiled tubes, the properties along the length of the coiled tube depend on hot rolled schedule at the steel supplier, sequence of coil splicing (since not all coils are equal), as well as the cold forming process at tube mill. The composite heat treated coiled tube is much more reliable than the standard coiled tube. For example, the properties of the composite heat treated coiled tube can be more consistent since the properties primarily depend on the heat treatment process while conventional coiled tubes have many variables that result in large variations in properties between sections of the coiled tube and also between different coiled tubes.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635

## 15

overall performance of the coiled tube. These property variations could not be generated during the hot rolling since the property changes are affected by the degree of reduction during rolling.

## Example 4

During hot rolling, the final properties are affected by the schedule of reduction at the hot rolling mill as well as the cooling at the run out table and final coiling process. Since the water in the run out table could generate differing cooling patterns across the width of the hot rolled coil, a faster cooling on coil edges and variations along the length due to "hot lead end practices" to facilitate coiling, as well as differential cooling of the inside of the coil with respect to the ends, the properties of the tubes would inherit these variations. In the case of the heat treated coiled tubes, the variation of properties are mainly affected by the chemistry and hence occur at a heat level (e.g., a heat size is the size of the ladle in the steelmaking process and hence is the maximum volume with same chemistry produced by a batch steelmaking process). The variation of properties of the composite heat treated coiled tube could be under control by having improved control of the heat treatment (heating, soaking, cooling, etc. (e.g., rate and time)) along the length of the coiled tube.

Although the foregoing description has shown, described, and pointed out the fundamental novel features of the present teachings, it will be understood that various omissions, substitutions, and changes in the form of the detail of the apparatus as illustrated, as well as the uses thereof, may be made by those skilled in the art, without departing from the scope of the present teachings. Consequently, the scope of the present teachings should not be limited to the foregoing discussion.

What is claimed is:

1. A method of heat treating a coiled tube, the method comprising:  
welding a plurality of steel strips together end to end to form a plurality of welded strips and longitudinally welding the plurality of strips to form a tube with a substantially constant inner diameter, outer diameter, and wall thickness along at least a first portion, a second portion and a third portion, the third portion being disposed between the first portion and the second portion;  
coiling the tube on a spool to form the coiled tube;  
uncoiling the coiled tube from the spool to obtain an uncoiled tube with the at least a first portion, the second portion and the third portion;  
selecting at least one predetermined parameter to be varied during a continuous quench and temper heat treatment process;  
after uncoiling the coiled tube, performing the continuous quench and temper heat treatment process along the first portion, the second portion and the third portion, wherein the at least one predetermined parameter of the continuous heat treatment process applied to the first portion varies from the at least one predetermined parameter applied during the continuous heat treatment process to the third portion and the at least one predetermined parameter of the continuous heat treatment process applied to the third portion varies from the at least one predetermined parameter of the continuous heat treatment process applied to the second portion to thereby modify a microstructure of the uncoiled tube and thereby resulting in a composite uncoiled tube with

## 16

the first portion having a greater post-heat-treatment yield strength value than a post-heat-treatment yield strength value of the third portion and the third portion having a greater post-heat-treatment yield strength value than a yield strength value of the second portion, and wherein the composite uncoiled tube after the continuous heat treatment process has a tempered martensite microstructure in the first, second and third portions of the uncoiled tube; and  
re-coiling the composite uncoiled tube after performing the continuous quench and temper heat treatment process;  
wherein the post-heat-treatment yield strength values are between 80 and 140 ksi.

2. The method of claim 1, wherein the coiled tube has a substantially uniform steel composition along the first portion, the second portion, and the third portion.
3. The method of claim 1, wherein the performing the continuous quench and temper heat treatment process comprises translating the uncoiled coiled tube through a heat treatment system that performs heating action, cooling action, or both.
4. The method of claim 3, wherein the translating the uncoiled tube is at variable speeds.
5. The method of claim 1, wherein the performing a continuous quench and temper heat treatment process comprises at least one quenching operation, intermediate operation, and tempering operation.
6. The method of claim 1, wherein the at least one predetermined parameter of the continuous heat treatment process is selected from a group consisting of temperature, soak time, heating rate, and cooling rate.
7. The method of claim 6, wherein the at least one predetermined parameter of the continuous heat treatment process that is varied comprises at least two of temperature, soak time, heating rate, and cooling rate.
8. The method of claim 1, wherein the coiled tube has a first end configured to be positioned at an upper portion of a wellbore and a second end configured to be positioned at an lower portion of the wellbore and post-heat treatment yield strength decreases with distance from the first end.
9. The method of claim 1 wherein the first portion is configured to be positioned at a top of a wellbore and has a length of at least 1000 feet and the second portion is configured to be positioned toward a bottom of the wellbore relative to the first portion and has a length of at least 1,500 feet and the third portion has a length of at least 1,500 feet and a total length of the coiled tube is between 10,000 and 40,000 feet.
10. The method of claim 1, wherein the first portion is adjacent to the third portion and the second portion is adjacent to the third portion.
11. The method of claim 1, wherein the continuous heat treatment process results in at least one post-heat treatment property being selected from a group consisting of mechanical properties, corrosion resistance, and microstructures.
12. The method of claim 11, where the mechanical property is selected from a group consisting of yield strength, ultimate tensile strength, elastic modulus, toughness, fracture toughness, fatigue life, fatigue strength, grain size, and hardness.
13. The method of claim 1, wherein the composite uncoiled tube after the continuous heat treatment process has a uniformity of microstructure.
14. The method of claim 1, further including providing the steel strips for welding into the tube, wherein the steel strips

## 17

include from about 0.010 wt % to about 0.025 wt % titanium and from about 0.0010 wt % to about 0.0025 wt % of boron.

**15.** A method of heat treating a tube, the method comprising:

welding a plurality of steel strips together end to end to form a plurality of welded strips and longitudinally welding the plurality of strips to form a tube with a substantially constant inner diameter, outer diameter, and wall thickness along at least a first portion, a second portion and a third portion, the third portion being disposed between the first portion and the second portion; and

selecting at least one predetermined parameter to be varied during a continuous quench and temper heat treatment process;

after forming the tube, performing the continuous quench and temper heat treatment process along the first portion, the second portion and the third portion, wherein the at least one predetermined parameter of the continuous heat treatment process applied to the first portion varies from the at least one predetermined parameter applied during the continuous heat treatment process to the second portion and the at least one predetermined parameter of the continuous heat treatment process applied to the third portion varies from the at least one predetermined parameter of the continuous heat treatment process applied to the second portion to thereby modify a microstructure of the tube and thereby resulting in a composite tube with the first portion having a greater post-heat-treatment yield strength value than a post-heat-treatment yield strength value of the third portion and the third portion having a greater post-heat-treatment yield strength value than a yield strength value of the second portion, and wherein the composite tube after the continuous heat treatment process has a tempered martensite microstructure in the first, second and third portions of the uncoiled tube;

wherein the post-heat-treatment yield strength values are between 80 and 140 ksi.

**16.** The method of claim 15, wherein the tube has a substantially uniform steel composition along the first portion, the second portion, and the third portion.

**17.** The method of claim 15, wherein performing the continuous quench and temper heat treatment process comprises translating the tube through a heat treatment system that performs heating action, cooling action, or both.

## 18

**18.** The method of claim 17, wherein translating the tube is at variable speeds.

**19.** The method of claim 15, wherein the performing a continuous quench and temper heat treatment process comprises at least one quenching operation, intermediate operation, and tempering operation.

**20.** The method of claim 15, wherein the at least one predetermined parameter of the continuous heat treatment process is selected from a group consisting of temperature, soak time, heating rate, and cooling rate.

**21.** The method of claim 15, wherein the at least one predetermined parameter of the continuous heat treatment process that is varied comprises at least two of temperature, soak time, heating rate, and cooling rate.

**22.** The method of claim 15, wherein the tube has a first end configured to be positioned at an upper portion of a wellbore and a second end configured to be positioned at an lower portion of the wellbore and post-heat treatment yield strength decreases with distance from the first end.

**23.** The method of claim 15, wherein the first portion is configured to be positioned at a top of a wellbore and has a length of at least 1,000 feet and the second portion is configured to be positioned toward a bottom of the wellbore relative to the first portion and has a length of at least 1,500 feet and the third portion has a length of at least 1,500 feet and a total length of the coiled tube is between 10,000 feet and 40,000 feet.

**24.** The method of claim 15, wherein the continuous heat-treatment process results in least one property selected from a group consisting of mechanical properties, corrosion resistance, and microstructures.

**25.** The method of claim 24, where the mechanical property is selected from a group consisting of yield strength, ultimate tensile strength, elastic modulus, toughness, fracture toughness, fatigue life, fatigue strength, grain size, and hardness.

**26.** The method of claim 15, wherein the composite tube after the continuous heat treatment process has a uniformity of microstructure.

**27.** The method of claim 15, further including providing the steel strips for welding into the tube, wherein the steel strips include from about 0.010 wt % to about 0.025 wt % titanium and from about 0.0010 wt % to about 0.0025 wt % of boron.

**28.** The method of claim 15, wherein the first portion is adjacent to the third portion and the second portion is adjacent to the third portion.

\* \* \* \* \*